

1

3,482,927  
METHOD FOR IMPARTING ANTIVESICANT  
PROPERTIES TO FABRIC

Samuel J. O'Brien, Dunellen, Michael T. Beachem, Somerset, and Frederic H. Megson, Martinsville, N.J., assignors, by mesne assignments, to the United States of America as represented by the Secretary of the Army  
No Drawing. Filed Jan. 24, 1967, Ser. No. 611,481  
Int. Cl. D06m 13/34

U.S. CL. 8—116.3

3 Claims

## ABSTRACT OF THE DISCLOSURE

A method for imparting antivesicant properties to fabrics comprising the contacting of the fabric with a derivative of 8-quinolinol, and further contacting said treated fabrics with a metal salt.

The present invention relates to an improved method for imparting antivesicant properties to cellulosic fabrics and more particularly to imparting antivesicant properties to cellulosic fabrics by impregnating or modifying them with metal chelates of 8-hydroxyquinoline and derivatives thereof.

Vesicant agents, such as mustard gas, attack the skin as well as the respiratory system of exposed personnel. Therefore, a body shield, in addition to a protective mask, is essential to prevent casualties. A fabric impermeable to all fluids would afford complete protection, but would be impractical, especially in warm climates, for extended periods of wear. More preferable is protection built into occupational clothing; thereby permitting air circulation and preventing moisture accumulation.

Mustard gas is the term applied to the well-known vesicant, bis(2-chloroethyl) sulfide; in its standard form as vapor or as air borne droplets. Various processes and compounds have been suggested and employed to impart finishes to the fabric used for military uniforms which would deactivate mustard gas and would prevent its passage through the cloth. But the efficiency of prior methods leaves much to be desired. For example, among the most commonly used are the N-chloroamides. Once on the fabric, these compounds lose activation by hydrolysis by atmospheric moisture, by perspiration, by thermal decomposition, and by the like.

The present invention is premised on the discovery that cellulosic fabrics treated with metal chelates of 8-hydroxyquinoline have useful and superior characteristics for imparting antivesicant properties to fabrics, especially against mustard gas. Accordingly, it is among the objects of the present invention to provide a treatment for air-permeable cellulosic fabric materials that will prevent passage of vesicant agent vapors through the garment. It is a further object to provide a permanent, noninjurious finish for such fabric materials which requires no further treatment by the wearer for antivesicant protection. It is a final object to provide a vesicant-resistant treatment for textile fabrics that is relatively stable and that does not adversely affect the tensile strength of the fabric. These and other objects and advantages of the instant invention will be fully apparent from the following description and examples.

An antivesicant capacity may be imparted to any fabric by simply padding a solution or dispersion of copper 8-quinolinolate thereon and drying the fabric. The padding process itself involves submerging the fabric in the solution, permitting it to soak for a few minutes, and gently squeezing it between rollers. In such a manner the wet weight of the fabric can be increased by 50%.

2

Fabrics providing a cellulosic substrate are conducive to more permanent protection fixation. In fact, any substrates having active hydrogen atoms are suitable; for example, polyvinyl alcohol, modified starches and the like.

To obtain more durable antivesicant protection, it is desirable to "fix" catalytically a fiber reactive quinoline derivative to the fabric and treat the thus modified fabric further with a metal salt to form a metal chelate. The metal chelate becomes an integral, chemically-bonded part of the fabric. Especially suitable for the latter process are the 5-hydroxymethyl and the 5,7 bis (hydroxymethyl) derivatives of 8-hydroxyquinoline. The process is represented by the following reaction:



where "cell" designates a portion of the cellulose chain of the fabric. The last configuration may represent any or all of the following structures:



Compounds useful in the process of the invention may be defined as metal chelates of compounds represented by the formula:



where  $R_1$  and  $R_2$  are hydrogen or  $CH_2OH$  or both. The compounds, represented by the last formula, where at least one of the  $R$ 's is  $CH_2OH$  are useful in the method of application wherein the compound is first bonded to the fabric with a catalyst and then chelated with a metal. The hydroxymethylquinoline derivatives are prepared by reaction with formaldehyde.

To accomplish the fixation on the fabric, typical acid catalysts, well known in the textile chemical and textile resin finish arts, are used. Examples are zinc nitrate magnesium chloride and acid salts of amines. Copper nitrate used in excess will catalyze fixation and react to form the chelate in one operation.

Although copper is the preferred metal for chelate formation, other metals known to react with 8-hydroxyquinoline can be used. Found suitable were chromium,

silver, iron, mercury, nickel, zinc, aluminum, and cobalt; some of which may be employed in more than one valence state, e.g. cuprous and cupric. Additionally, compounds of these metals impart to the fabric in durable, fiber-reacted form other useful properties of the metal or of the metal coordination complex. For instance, copper will add fungicidal, aluminum will add antiperspirant, and mercury will add bactericidal activity. The 8-hydroxyquinoline itself is effective to some degree as an antivesicant, although known previously as an antifungal agent.

After bonding the methylol derivatives of 8-hydroxyquinoline to the fabric, copper complexes may be formed using other copper complexes such as copper ethylenediamine nitrate and copper diethanolamine nitrate, depicted structurally below:



The copper provided by these complexes affords additional antivesicant activity.

Chemically bonding the quinoline moiety to the cellulose affords the durable antivesicant finish unobtainable by simple padding. The structure of the coordination compound can take a variety of forms, provided it is capable of having a fiber reactive group attached to it. Organic coordination compounds which will work are dihydric alcohols, alkanolamines, amino acids acetylacetones, cyclic acids, hydroxybenzoic acids, thiosemicarbazones, guanidines, dicyandiamides, aminothiophenols, hetero-N, -O and -S compounds, azophenols, nitriles, salicylaldehydes, aldimines, oximes, and so on. Any free orbitals remaining after combining the metal atom with the coordination compound are filled by other groups from the substrate (e.g. hydroxyls of cellulose) or by adding on small molecules like NH<sub>3</sub> or H<sub>2</sub>O.

The efficiency of the mustard-gas barrier is determined by the "Dawson Test" a measurement of the percent of mustard gas, initially present in an air stream, retained on a fabric after air passage through the fabric. In the examples which follow, the preparations of the antivesicant complexes and treatment of the fabric are described. Table 1, following the last example shown hereinafter, depicts the Dawson Test results. It will be observed that the process whereby 8-hydroxyquinoline-5-methylol derivatives are fixed to the fabric and then "topped" with a metal compound solution to form the chelates is significantly more effective than hydroxyquinolinemethanol derivatives alone.

#### EXAMPLE I

A 10% solution of a commercially available fungicidal preparation of copper 8-quinolinolate in a hydrocarbon vehicle is padded onto cellulosic fabric.



#### EXAMPLE II

With the aid of about 0.1 part of 75% solution of a surfactant (Aerosol OT-diethyl sodium sulfosuccinate), 100 parts of pulverized 8-quinolinol is dispersed in 500 parts of water. Six parts by volume of aqueous sodium hydroxide solution (10 g./100 ml. concn.) is added to make the mixture moderately alkaline to phenolphthalein

indicator. While stirring the mixture at 25-30° C., 230 parts of a 36% aqueous solution of formaldehyde is added over 10-15 minutes. After stirring overnight at 25-30° C., the slurry is filtered, and the solid is washed with three portions of 250 parts by volume of water, dried overnight at 55-60° C., and ground until the material can be passed through a 60-mesh screen.

The pale orange solid obtained amounts to 117 parts and analyzes C<sub>10.5</sub>H<sub>10.9</sub>N<sub>1.0</sub>; indicating it consists of monomethylolated and dimethylolated products in approximately equal molar amounts. On the basis of the known chemistry of 8-quinolinol these products are primarily 8-hydroxy-5-quinolinemethanol, and 8-hydroxy-5,7-quinolinedimethanol and 8-hydroxy-5,7-quinolinemethanol.

Cotton sateen fabric is padded with a dimethylformamide solution containing 20% of the above compound and 2% zinc nitrate (the latter added as an aqueous solution), dried two minutes at 225° F., and cured three minutes at 350° F. The resulting fabric is processed washed one complete cycle (in a typical household washing machine) at 160° F. using 0.1% Tide detergent and 0.1% soda ash, and is air dried.

A portion of the above fabric is "topped" with copper nitrate by padding it with a 20% solution of Cu(NO<sub>3</sub>)<sub>2</sub> in water, air drying it, rewashing it at 160° F. with plain water, and again air drying it. Analysis of the fabric now shows a Cu/N atomic ratio of 0.6 (theory 0.5) and a concentration of metal chelate (based on the Cu content) of 6.7% of the weight of the fabric.

#### EXAMPLE III

To a mixture of 79.8 parts of 8-quinolinol (pulverized until all passes through a 60-mesh screen), 0.1 part of a surfactant solution (Aerosol OT) and 5 parts by volume of aqueous sodium hydroxide solution (20 g./100 ml. concn.) in 500 parts by volume of water, is added rapidly with good stirring 91.8 parts of 36-38% aqueous formaldehyde solution. At this point the pH is about 9. After stirring overnight at 25-30° C., the solid is filtered off, washed twice with water, and dried overnight at 50-55° C. The cream colored solid amounts to 92.8 parts (96% of theory).

The compound is fixed on cotton sateen fabric, washed, and dried as in Example II. Next, the treated fabric is soaked for about two hours in 20% solution (on an anhydrous basis) of cupric chloride, run through a padder, and air dried.

The above process is repeated exactly with 20% solutions of the following salts substituted for the cupric chloride:

|                  |                  |
|------------------|------------------|
| chromium sulfate | nickel salt      |
| silver nitrate   | cuprous chloride |
| ferric sulfate   | zinc salt        |
| mercuric nitrate | cobalt salt      |

#### EXAMPLE IV

To 160.0 parts of 8-quinolinol in 1000 parts by volume of water containing 0.2 part by volume of a 25% aqueous solution of a surfactant (Aerosol OT) and 10 parts by volume of aqueous sodium hydroxide solution (20 g./100 ml. concn.), is added 184.0 parts of aqueous formaldehyde solution (36-38%) and the mixture is stirred for 18 hours. The product filtered off, washed with water and dried at 50-55° C., amounts to 192.1 (99% of theory) of cream white solid analyzing C<sub>10.4</sub>H<sub>9.4</sub>N<sub>1.0</sub> (calculated for 8-hydroxy-5-quinoline methanol-C<sub>10</sub>H<sub>9</sub>NO<sub>2</sub>).

Fabric is padded with a solution containing 20.0 parts of the above and 30.4 parts of Cu(NO<sub>3</sub>)<sub>2</sub>·3H<sub>2</sub>O, dried two minutes at 225° F., cured three minutes at 350° F., washed in plain water and air dried.

#### EXAMPLE V

Fabric is padded with a solution containing 20% 8-hydroxy-5-quinoline methanol (prepared in Example IV) and

2%  $Zn(NO_3)_2$ , dried two minutes at 225° F., cured three minutes at 350° F., washed in a household washing machine at 160° F. using 1% Tide detergent and 1% soda ash, and air dried. A portion of the thus treated fabric is padded with 20% solution of  $Cu(NO_3)_2$ , air dried, and washed in plain water. Another portion is padded with 20% solution of  $Cu(NH_2CH_2CH_2OH)_2(NO_3)_2$ , air dried, and washed in plain water. And a third portion is padded with 20% solution of  $Cu(NH_2CH_2CH_2NH_2)(NO_3)_2$ , air dried, but not washed. As a control, a piece of untreated fabric is padded with the last named solution and air dried.

5

10

What is claimed is:

1. An improved method for imparting antivesicant properties to cellulosic fabrics comprising the steps of: padding said fabric with a derivative formed by the reaction of 8-quinolinol and an aqueous solution of formaldehyde in the presence of a catalyst in order to fix said derivative to the fabric drying, and further contacting said modified fabric with a metal salt to form a metal chelate.
2. A method in accordance with claim 1 wherein the 8-quinolinol derivative is selected from the group consisting of 8-hydroxy-5-quinolinemethanol, 8-hydroxy-5,7-quinolinemethanol, and 8-hydroxy-5,7-quinolinedimethanol.

TABLE I

| Test run    | Compound applied                                                                                         | Application Method | Percent mustard retention |          |          |
|-------------|----------------------------------------------------------------------------------------------------------|--------------------|---------------------------|----------|----------|
|             |                                                                                                          |                    | 0-2 hrs.                  | 2-4 hrs. | 4-6 hrs. |
| Example I   | Copper 8-quinolinolate                                                                                   | Padded             | 88                        | 58       | 41       |
| Example II  | 8-hydroxy-5-quinolinemethanol                                                                            | Fixed (no metal)   | 14                        |          |          |
|             | 8-hydroxy-5-quinolinemethanol, copper salt                                                               | Fixed              | 73                        | 53       | 51       |
| Example III | 8-hydroxy-5-quinolinemethanol, copper salt<br>(from $CuCl_2$ )                                           | do                 | 49                        | 41       | 39       |
|             | 8-hydroxy-5-quinolinemethanol, chromium salt                                                             | do                 | 36                        | 26       | 24       |
|             | 8-hydroxy-5-quinolinemethanol, cerium salt                                                               | do                 | 42                        | 33       | 30       |
|             | 8-hydroxy-5-quinolinemethanol, silver salt                                                               | do                 | 42                        | 33       | 32       |
|             | 8-hydroxy-5-quinolinemethanol, ferric salt                                                               | do                 | 57                        | 40       | 38       |
|             | 8-hydroxy-5-quinolinemethanol, mercuric salt                                                             | do                 | 60                        | 54       | 51       |
| Example IV  | 8-hydroxy-5-quinolinemethanol, copper salt,<br>fixed with copper nitrate                                 | do                 | 51                        | 42       | 38       |
| Example V   | 8-hydroxy-5-quinolinemethanol,<br>8-hydroxy-5-quinolinemethanol, copper dietha-<br>nolamine nitrate salt | Fixed (no metal)   | 49                        | 33       | 31       |
|             | 8-hydroxy-5-quinolinemethanol, copper ethyl-<br>enediamine nitrate salt                                  | Fixed              | 65                        | 39       | 34       |
|             | Copper ethylenediamine nitrate                                                                           | do                 | 79                        | 61       | 46       |
|             | Copper ethylenediamine nitrate                                                                           | Padded             | 25                        |          |          |

While only preferred forms of the invention are described, other forms of the invention are contemplated and numerous changes and modifications may be made therein without departing from the spirit of the invention. 35

3. A method in accordance with claim 2 wherein the metal salts is selected from the group consisting of: cuprous chloride, copper, nitrate, chromium sulfate, silver nitrate, ferric sulfate, mercuric nitrate and zinc nitrate.

## References Cited

## UNITED STATES PATENTS

|           |         |                   |             |
|-----------|---------|-------------------|-------------|
| 2,250,660 | 7/1941  | Straub et al.     | 260—289     |
| 2,381,863 | 8/1945  | Benignus          | 117—138.5   |
| 2,698,263 | 12/1954 | Weick             | 117—138.5   |
| 2,721,824 | 10/1955 | Feigin et al.     | 260—270 X   |
| 3,033,865 | 5/1962  | Fronmuller et al. | 117—138.5 X |
| 3,088,916 | 5/1963  | Roman             | 252—106     |

WILLIAM D. MARTIN, Primary Examiner

T. G. DAVIS, JR., Assistant Examiner

U.S. Cl. X.R.

117—62.1, 118, 121, 143